

## UNITED STATES PATENT OFFICE

2,378,341

## DIESEL FUEL

William E. Vaughan and Frederick F. Rust,  
Berkeley, Calif., assignors to Shell Development  
Company, San Francisco, Calif., a corporation  
of Delaware

No Drawing. Application February 8, 1943,  
Serial No. 475,215

11 Claims.

(Cl. 44—57)

This invention relates to Diesel fuels containing a knock depressor, and more particularly deals with such fuels containing a small amount of a peroxide of a branched chain aliphatic hydrocarbon.

It is known that hydrocarbon peroxides and other organic peroxides have the property, when dissolved in hydrocarbon Diesel fuels, of acting as ignition accelerators of the latter, i. e., they increase the tane numbers of the fuel. However, the various peroxides used in the past for this purpose have had various disadvantages, among them being particularly their explosibility. For example, tetraline peroxide, ketone peroxides, etc., are all highly explosive, and their handling is exceedingly dangerous unless they are highly diluted with inert material. Other Diesel knock depressors, such as alkyl nitrates or dialkyl polysulfides, are either corrosive or produce corrosive products upon combustion or both. In contrast, the peroxides of this invention are substantially non-corrosive, stable and substantially non-explosive, even in highly concentrated state. On ignition, they burn with a sooty smooth flame, and when dropped on a hot plate maintained at 250° C., they merely vaporize, but fail to explode.

It is thus a purpose of this invention to produce Diesel fuel oils of increased cetane numbers, which are safe in manufacturing and handling. Another purpose is to provide a cheap and effective means for raising the cetane numbers of Diesel fuels.

Our invention comprises hydrocarbon Diesel fuels of relatively high cetane numbers containing an added small amount, i. e., about 1/4%—5%, and preferably 1%—3%, of peroxide of a hydrocarbon having an aliphatic tertiary carbon atom, wherein the peroxy radical connects two tertiary carbon atoms.

The peroxides used in this invention are produced by slow, non-explosive oxidation of a hydrocarbon containing at least one tertiary carbon atom of aliphatic character in the presence of a hydrogen halide, particularly hydrogen bromide, or a compound capable of yielding such hydrogen halide under operating conditions. Hydrocarbons of the above type may be represented by the formula



wherein each R represents a like or different alkyl, aryl, aralkyl, alicyclic or heterocyclic radi-

cal, two of which may together form an alicyclic ring, and which radicals may be further substituted, for instance, by the presence of one or more halogen, nitrogen or oxygen atoms which are attached to one or more of the carbon atoms of such radicals. A preferred class of organic compounds which may be used as a starting material comprises the saturated aliphatic hydrocarbons containing at least one tertiary carbon atom. Specific examples of the latter are isobutane, 2-methyl butane, 2-ethyl butane, 2-methyl pentane, 3-methyl pentane, 2,3-dimethyl butane, 2,4-dimethyl butane and their homologues, preferably having not more than about 12 carbon atoms.

The temperature of the oxidation is normally in the neighborhood of around 150° C., temperatures between 100° to about 250° C. being normally applicable.

The oxidation may be effected in the liquid or vapor phase or both, vapor phase being preferred.

As a result of the oxidation, some acids, ketones and aldehydes are produced; however, a substantial portion of the reaction product consists of the peroxides employed in this invention, which, it is believed, may be represented by the formula:



wherein each R again represents a like or different hydrocarbon radical which may or may not be further substituted. Preferred compounds

are the symmetrical, saturated, di(tertiary alkyl) peroxides having not more than about 24 carbon atoms. These compounds are water-white, oil-soluble, water-insoluble liquids having a pleasant odor. The peroxide obtained in the controlled oxidation of isobutane boils at 108°—110° C.

Mixtures of different peroxides may be used, such as may be obtained, for example, by oxidizing a mixture of isobutane and isopentane, or a mixture of several iso-octanes resulting from the polymerization of butylenes and hydrogenation of the polymers, or resulting from the alkylation of isobutane with butylenes, or other alkylate gasolines having relatively wide boiling ranges.

Also mixtures of hydrocarbons containing an aliphatic tertiary carbon atom with other hydrocarbons may be oxidized to produce the peroxides useful in accordance with this invention.

If desired, the Diesel fuels may contain additional additives, such as anti-oxidants, e. g.,

various alkyl phenols such as xylenols, trimethyl phenol, 2,4-dimethyl-6-tertiary butyl phenol, 4-methyl-2,6-ditertiary butyl phenol, etc.; aromatic amines, preferably secondary aromatic amines, such as N,N' dibutyl phenylene diamine, diphenylamine, phenyl alpha naphthylamine, alpha alpha', alpha beta, or beta beta' dinaphthylamines; amino phenols, such as benzyl para amino phenol, etc.; anti-corrosive agents such as dicarboxylic acids having at least 16 carbon atoms, e. g., alkyl succinic acids; pour point reducers, viscosity or viscosity index improvers, wear reducers, such as carbamic acid esters, allophanic acid esters, etc.

Moreover, other Diesel knock depressors, such as alkyl nitrates or nitrites, dialkyl tetra sulfides, etc., may be used in conjunction with the peroxides of this invention.

Knock rating improvements vary somewhat with the type of fuel to which the peroxides are added, the example below illustrating the improvement in cetane number when adding a peroxide of this invention to a specific Diesel fuel.

*Example*

To a California Diesel fuel having a cetane number of 40.5 was added 1% of isobutane peroxide prepared by the slow combustion described above. The cetane number of the fuel was thereby raised to slightly above 56.

We claim as our invention:

1. A Diesel fuel of improved cetane number comprising a predominant amount of a hydrocarbon Diesel fuel and a cetane improving amount of a peroxide of a hydrocarbon having at least one aliphatic tertiary carbon atom, the peroxy radical in said peroxide connecting two tertiary carbon atoms.

2. A Diesel fuel of improved cetane number comprising a predominant amount of a hydrocarbon Diesel fuel and a cetane improving amount of a peroxide of a chlorinated hydrocarbon having at least one aliphatic tertiary carbon atom, the peroxy radical in said peroxide connecting two tertiary carbon atoms.

3. A Diesel fuel of improved cetane number comprising a predominant amount of a hydrocarbon Diesel fuel containing about 1/4%-5% of a peroxide of a hydrocarbon having at least one aliphatic tertiary carbon atom, the peroxy radical in said peroxide connecting two tertiary carbon atoms.

4. A Diesel fuel of improved cetane number comprising a predominant amount of a hydrocarbon Diesel fuel containing about 1%-3% of a peroxide of a hydrocarbon having at least one aliphatic tertiary carbon atom, the peroxy radical in said peroxide connecting two tertiary carbon atoms.

5. A Diesel fuel of improved cetane number comprising a predominant amount of a hydro-

carbon Diesel fuel and a cetane improving amount of a peroxide of a hydrocarbon having not more than 12 carbon atoms and at least one aliphatic tertiary carbon atom, the peroxy radical in said peroxide connecting two tertiary carbon atoms.

6. A Diesel fuel of improved cetane number comprising a predominant amount of a hydrocarbon Diesel fuel and a cetane improving amount of a peroxide of compounds having the formula



wherein the several R's represent hydrocarbon radicals, the peroxy radical of said peroxide connecting two of said compounds through their tertiary carbon atoms.

7. A Diesel fuel of improved cetane number comprising a predominant amount of a hydrocarbon Diesel fuel and a cetane improving amount of a peroxide obtained by slow oxidation of a hydrocarbon containing at least one aliphatic tertiary carbon atom.

8. A Diesel fuel of improved cetane number comprising a predominant amount of a hydrocarbon Diesel fuel and a cetane improving amount of a peroxide having the formula



wherein the several R's represent hydrocarbon radicals.

9. A Diesel fuel of improved cetane number comprising a predominant amount of a hydrocarbon Diesel fuel and a cetane improving amount of a symmetrical peroxide having not more than 24 carbon atoms and the formula



wherein the several R's represent hydrocarbon radicals.

10. A Diesel fuel of improved cetane number comprising a predominant amount of a hydrocarbon Diesel fuel oil and a cetane improving amount of a di-isobutane peroxide wherein the peroxy radical connects two tertiary carbon radicals.

11. A Diesel fuel of improved cetane number comprising a predominant amount of a hydrocarbon Diesel fuel oil and a cetane improving amount of di-isopentane peroxide wherein the peroxy radical connects two tertiary carbon radicals.

WILLIAM E. VAUGHAN.  
FREDERICK F. RUST.

CERTIFICATE OF CORRECTION.

Patent No. 2,378,341.

June 12, 1945.

WILLIAM E. VAUGHAN, ET AL.

It is hereby certified that error appears in the printed specification of the above numbered patent requiring correction as follows: Page 1, first column, line 10, for "tane" read --cetane--; and that the said Letters Patent should be read with this correction therein that the same may conform to the record of the case in the Patent Office.

Signed and sealed this 23rd day of October, A. D. 1945.

Leslie Frazer

(Seal)

First Assistant Commissioner of Patents.